# EUROPEAN PATENT SPECIFICATION

(11) **EP 2 955 241 B1**
(45) Date of publication and mention of the grant of the patent: **24.01.2024**
(21) Application number: 14172142.3
(22) Date of filing: 12.06.2014
(51) Int. Cl.: C22C 29/08, B22F 1/00, C22C 29/06, C22C 29/10, C22C 29/16, B22F 3/22, C22C 1/051, B22F 1/10, B22F 5/00

(54) **Method for manufacturing a cemented carbide or cermet body**
Verfahren zur Herstellung von Hartmetallkörper oder Cermetkörper
Procédé pour la fabrication de pièces en carbures cémentés ou en cermet

(43) Date of publication of application: 16.12.2015
(73) Proprietor: Maschinenfabrik Gustav Eirich GmbH & Co. KG, 74736 Hardheim (DE)
(72) Inventor: Thompson, Christopher, Stafford, ST16 1EX (GB); Fuller, Peter George, Coventry, CV4 7DN (GB); Ronnheden, Sofia Maria, 13 755 Tungelsta (SE); Gerl, Stefan, 97956 Werbach (DE)
(74) Representative: WSL Patentanwälte Partnerschaft mbB

(56) References cited:
- EP-A1- 0 471 123
- EP-A1- 2 647 731
- CN-A- 101 892 409
- JP-A- 2012 052 237
- US-A- 4 478 888
- US-A- 4 610 931
- US-A- 5 619 000
- US-A1- 2003 124 017

## Description

### Technical Field

The present invention relates to new method of manufacturing a cemented carbide and/or a cermet wherein the cemented carbide and/or cermet has a microstructure with improved homogeneity.

### Background of the invention

Cemented carbide or cermet is commonly used for rotary tools as it has good wear properties.

In order to achieve optimal properties, the microstructure needs to contain as few clusters of enlarged hard metal grains as possible and also as few binder lakes as possible and additionally as little porosity as possible. EP 1724363 A1 discloses the wet milling of a powder mixture containing hard constituent powder(s) based on carbides of Ti, Zr, Hf, V, Nb, Ta, Cr, Mo and/or W and >15 wt% binder phase powder(s) of Co and /or Ni as well as pressing agents and spray drying. 0.05-0.50 wt% of a complex forming and/or pH-increasing/decreasing additive, such as triethanolamine, hydroxides or acids, and a thickener in an amount of 0.01 - 0.10 wt% is added to the powder mixture before milling.

US5922978 A discloses a pressable powder being formed by a method comprising mixing, in essentially deoxygenated water, a first powder selected from the group consisting of a transition metal carbide and transition metal with an additional component selected from the group consisting of a second powder comprised of a transition metal carbide, transition metal or mixture thereof; an organic binder and combination thereof and drying the mixed mixture to form the pressable powder, wherein the second powder is chemically different than the first powder. The pressable powder may then be formed into a shaped part and subsequently densifed into a densifed part, such as a cemented tungsten carbide and triethanolamine could be added as a corrosion inhibitor.

US6878182 B2 discloses a slurry based on ethanol-water and contains metal carbide and metallic raw materials as well as stearic acid and a low concentration of polyethylenimine (PEI). The concentration of PEI is 0.01-1 wt % of the raw material weight.

EP1153652 A1 discloses a procedure of mixing WC and Co with additional constituents suitable for making cemented carbides, with water, ethanol or mixtures of ethanol and water, and a polyethylenimine-based dispersant to achieve a well dispersed suspension suitable for spray drying. The method is characterised in adding to the slurry as dispersant 0.1-10 wt%, preferably 0.1-1 wt%, of a polyethylenimine-based polyelectrolyte.

US 4,478,888 is directed to a process for producing a carbide grade powder mixture for making a cemented metal carbide, wherein in this process a mixture of metal carbide particles and wax is formed at a temperature above the melting point of the wax.

JP 2012 052237 A discloses a method for producing a cemented carbide having high transverse strength with less variation, and a rotating tool of the cemented carbide having excellent breakage resistance even when used for small diameter drilling or high-feed cutting.

EP 2 647 731 A1 discloses a method for producing a cemented carbide, wherein acoustic waves are used in order to achieve a homogenous mixture of a powder blend.

EP 0 471 123 A1 is directed to a process for preparing an inorganic article by mixing an inorganic powder, water and a dispersant in a slurry, heating the blend, admixing the heated blend with a thermally gelable polymeric binder at a temperature above the gelation point of the polymer to form a slurry mixture and cooling the mixture before extruding articles by extruding the mixture.

US 5,619,000 discloses a method of producing a sintered body comprising one or more hard constituents and a binder phase based on cobalt, nickel and/or iron by powder metallurgical methods milling, pressing and sintering of powders.

CN 101 892 409 A is directed to a method for preparing a milling coating hard alloy. The method comprises the following steps: adding a metal cobalt powder and a tantalum carbide powder into a tantalum carbide powder of which the particle size is between 4 and 6 µm and the total carbon is between 6.08 and 6.13 percent to prepare a mixture; performing compression molding and vacuum sintering on the mixture to prepare a high-intensity and high-toughness hard alloy substrate which consists of 10 to 13 weight percent of the metal cobalt powder, 1 to 3 weight percent of the tantalum carbide powder and 84 to 89 weight percent of the tungsten carbide powder; and performing grinding machining and cutting edge rounding treatment on the hard alloy substrate and performing physical vapor deposition (PVD) super nitrogen-titanium-aluminum-nitrogen coating treatment.

In all the above mentioned disclosures, except for the last, the dispersing agents, such as triethanolamine and/or polyethylenimine are added to a wet mixture or slurry. The problems with these methods are that mixing of the different constituents will be incomplete and the obtained products will therefore not have the desired homogenous microstructure when sintered and therefore not the desired properties step. The present invention will solve or at least reduce the above mentioned problems.

### Summary

In one aspect the present invention describes a method of manufacturing a cemented carbide and/or cermet comprising the steps of:
a) providing a powder comprising metal carbide(s) and binder metal(s) and optionally metal nitride(s);
b) mixing the powder composition provided by step a) under vacuum before
c) adding at least one organic binder to the powder composition;
d) mixing the at least one organic binder with the powder composition under vacuum and raising the temperature to a predetermined temperature and keeping the temperature for a predetermined time until the organic binder has melted;
e) subjecting the obtained mixture of step d) to forming and sintering processes;
wherein one or more dispersing agents is added to the powder composition in step a) and wherein one or more cooling agents is added to the powder composition in step b).

Hence, at least one dispersing agent is added to the dry powder mixture in the first step.

In another aspect of the present disclosure, not forming part of the invention, a cemented carbide or cermet body is obtained according to the hereinabove or hereinafter defined method, wherein the microstructure of the cemented carbide or the cermet has no clusters of hard metal grains with a diameter > 5 x the average hard metal grain size.

In another aspect , not forming part of the invention, a cemented carbide or cermet body obtained according to the method as defined herein above or hereinafter, which cemented carbide or cermet body is used for a rotary cutter or any other wear application

The method described hereinabove or hereinafter will provide a desired homogenous powder mixture which in turn will results in a product (cemented carbide and/or cermet) with more homogenous microstructure and therefore having improved properties, for example increased tensile strength, increased hardness, increased fracture toughness and/or increased wear resistance. This consequently will result in an improvement in the performance when the cemented carbide and/or cermet is used for a rotary cutter or wear part.

### Brief description of drawings

- Figure 1:: discloses optical micrograph showing microstructure of cemented carbide from test 1 showing an example of a hard metal cluster.
- Figure 2:: discloses optical micrograph showing microstructure of cemented carbide from test 1 showing an example of binder lakes.
- Figure 3:: discloses optical micrograph showing microstructure of cemented carbide from test 3
- Figure 4:: discloses optical micrograph showing microstructure of cemented carbide from test 8

All the optical micrographs were taken on Olymus PMG3-LSH-3 inverted microscope.

### Detailed description

The present invention describes a method of manufacturing a cemented carbide and/or cermet comprising the steps of:
a) providing a powder comprising metal carbide(s) and binder metal(s) and optionally metal nitride(s);
b) mixing the powder composition under vacuum;
c) adding at least one organic binder to the powder composition;
d) mixing the at least one organic binder with the powder composition under vacuum and raising the temperature to a predetermined temperature and keeping the temperature for a predetermined time until the organic binder has melted;
subjecting the obtained mixture of step d) to forming and sintering processes; wherein one or more dispersing agents is added to the powder composition in step a) and wherein one or more cooling agents is added to the powder composition in step b).

The method, in one aspect not forming part of the invention, preferably comprises making a dough for use in extrusion. In such a case, the method preferably comprises adding organic solvents (mono propylene glycol (MPG) and/or Oleic acid) to the mixture obtained so as to lubricate mixture prior to sintering in step e) above.

Additionally, according to the present method, the one or more dispersing agents is selected from triethanol amine (TEA) or polyethylene imine (PEI) or a mixture thereof.

Further, according to the present method as defined hereinabove or hereinafter, the powder provided in step a) comprises metal carbide(s) and binder metal(s) and metal nitride(s).

When adding at least one organic binder to the cemented carbide or cermet production process, a two-step mixing process is necessary. This is because if the metal carbide powder, the metal nitride powder, binder metal powder and organic binder(s) are mixed together in the single step, the organic binder will stick to the binder metal powder, which will prevent efficient mixing and consequently will provide a cemented carbide or cermet with a non-homogenous microstructure. The desired homogeneity of the microstructure of the cemented carbide or cermet is obtained by adding one or more dispersing agents to the powder composition thus ensuring that the composition is well mixed before the at least one organic binder is added. The present invention provides an effective method for obtaining cemented carbides and/or cermets having a homogenous mixture as the one or more dispersing agents is added to the first mixing step (step a) wherein powders of the metal carbide(s) and binder metal(s) and optionally metal nitride(s) are mixed in dry form. Thus, this mixing step is a dry mixing step having a moisture content of less than or equal to 5 wt% (based on the total powder composition). The mixing step is defined as dry in that no significant quantities of water and/or ethanol and/or any other solvent are added to produce a wet slurry. The only liquid added in this step is, if necessary, a small quantity liquid in the form of cooling agent. The cooling agent is selected from water, ethanol and any other suitable solvent which would readily evaporate under the mixing conditions. The temperature at this first mixing step needs to be maintained to below 50°C to avoid oxidation. The powder composition should be kept as dry as possible during this first mixing step, therefore the moisture content is less than or equal to 5 wt%. No cooling agent is added until the temperature starts to rise above 50°C and when the temperature starts to rise, the amount of cooling agent added should be as little as possible in order to keep the powder mixture as dry as possible, i.e. with a moisture content less than or equal to 5 wt%. During this step, the one or more dispersing agents are added. The addition of the one or more dispersing agents in this step ensures that the powders of metal carbide(s) and binder metal(s) and optionally metal nitride(s) are well mixed before the at least one organic binder is added in the second mixing step.

The one or more dispersing agents is selected from triethanol amine (TEA), polyethylene imine (PEI) or a mixture thereof. The amount of dispersing agent is of from 0.05 - 0.5 wt% of total powder mixture.

According to the present method, the cemented carbide comprises metal carbide(s) and/or metal nitride(s) in the range of from 70 to 97 wt% and binder metal(s) in the range of from 3 wt% to 30 wt% (the wt% is based on the total content of the cemented carbide). The metal carbide(s) and/or metal nitride(s) comprises more than or equal to70 wt% tungsten carbide and less than or equal 30 wt% of at least one other metal carbide and/or metal nitride selected from titanium carbide, titanium nitride, tantalum carbide, tantalum nitride, niobium carbide and a mixture thereof (the wt% is based on the total content of metal carbides and metal nitrides)

According to the present method, the cermet comprises metal carbide(s) and/or metal nitride(s) in the range of from 70 to 97 wt% and binder metal in the range of from 3 wt% to 30 wt% (the wt% is based on the total content of the cermet). Further, the cermet comprises a combination of one or more metal carbides and/or metal nitrides selected from titanium carbide, titanium nitride, tungsten carbide, tantalum carbide, niobium carbide, vanadium carbide, molybdenum carbide, chromium carbide and a mixture thereof, with the highest proportion being titanium based, i.e. the titanium is in the form of carbide and/or nitride and is in the range of from 30 to 60 wt% (the wt% is based on the total content of the cermet). Further, the cermet does not comprise any free hexagonal tungsten carbide. The cermet comprises tungsten carbide without any free hexagonal structure in the range of from 10 to 20 wt%. Hexagonal tungsten carbide has a structure made up of a simple hexagonal lattice of tungsten atoms layered directly over one another with the carbon atoms filling half the interstices giving both tungsten and carbon a regular trigonal prismatic structure.

The cermet and/or cemented carbide may also comprise small amounts, such as less than or equal to 3 wt% of other compounds e.g. MoC, VC, and/or Cr₃C₂.

According to one aspect of the invention, the binder metal(s) is selected from cobalt, molybdenum, iron, chromium or nickel and a mixture thereof.

According to the method as defined hereinabove or hereinafter, one or more organic solvents is optionally added in step d).

The method as defined herein above or hereinafter, optionally comprises that the obtained mixture of step d) is dried after the forming and prior to sintering in step e).

According to another aspect of the invention, the forming is performed by using extrusion, pressing operation or injection moulding.

In the first mixing stage, the metal carbide(s) and/or metal nitride(s) may be selected from the group of tungsten carbide, tantalum carbide, niobium carbide, titanium carbide, titanium nitride, tantalum nitride, vanadium carbide, molybdenum carbide, chromium carbide and mixture thereof. The binder metal(s) is any of one single binder metal or a blend of two or more metals or an alloy of two or more metals and the binder metal are selected from cobalt, molybdenum, iron, chromium or nickel. However, which carbides and/or nitrides that are selected and the proportions thereof depends on if the final product will be a cemented carbide or a cermet and the desired final properties of the final product.

Once the components of the first mixing step are well mixed one or more organic binders are added. The at least one organic binder used in the process as defined hereinabove or hereinafter is selected from polyethylene glycol (PEG), methyl cellulose (MC), wax systems such as petroleum wax, vegetable wax or synthetic wax, polyvinyl butyral (PVB), polyvinyl alcohol (PVA) and a mixture thereof. The organic binder could also be a mixture of the same organic binder but of different types e.g. a mixture of different PVA, PEG or MC.

In this second step, the mixing is continued under vacuum (to avoid trapped air in the mixture) until the temperature reaches approximately 70°C (or higher depending upon the organic binder) to ensure that organic binders have melted or are fully dispersed. If a dough is to be produced, for example if the cemented carbide or cermet is to be formed using an extrusion process, then additional wet organic solvents such as oleic acid , monopropylene glycol or water may also be added in the second mixing step. In this case, an additional drying step would be required after forming and prior to sintering.

According to the present method, the mixing may be performed by using a planetary mixer. A planetary mixer contains blades which rotate on their own axes, and at the same time on a common axis, thereby providing complete mixing in a short timeframe. The benefit of this type of mixer is that it means that compared to the conventional ball milling commonly used to mix powders to be used for obtaining cemented carbides and cermets, the mixing time is reduced and there is no attrition of the raw materials. Other high speed mixing devices could also be used for example high speed rotor.

In one aspect, not forming part of the invention, the cemented carbide or cermet obtained has a microstructure with no clusters of metal grains with a diameter > 5 x the average hard metal grain size. According to the method as defined hereinabove or hereinafter, the cemented carbide and/or cermet which is obtained thereby has a microstructure comprising no clusters of enlarged hard metal grains with a diameter greater than 5 x the average hard metal grain size and no more than 0.5 per cm². The average hard metal grain size is determined using the linear intercept method according to ISO standard 4499. A cluster is defined as 5 or more grains located next to each other. An example is shown in figure 1.

In another aspect, not forming part of the invention, the microstructure cemented carbide or cermet has no binder lakes with a diameter > 5 x the average hard metal grain size. Further, according to the method as defined hereinabove or hereinafter, the cemented carbide and/or cermet obtained thereby has a microstructure comprising no binder lakes with a diameter greater than 5 x the average hard metal grain size and no more than 0.5 cm per cm². A binder lake is defined as an area consisting of only binder with no hard metal grains in that region. An example is shown in figure 2.

In another aspect, not forming part of the nivention, the microstructure of the cemented carbide or cermet has A type porosity of A00 or A02. Additionally, according to the method as defined hereinabove or hereinafter, the cemented carbide and/or cermet body obtained thereby has a microstructure with A type porosity of A00 or A02. Porosity is measured according to ISO standard 4505. A type porosity is defined as voids less than 10 µm in diameter. A00 corresponds to the total absence of any porous volume and A02 means a maximum volume of A type pores of 0.02% of the total material volume.

In another aspect, not forming part of the invention, the cemented carbide or cermet may be used for a rotary cutter or any other wear application. The cemented carbide or cermet body obtained from the method as defined hereinabove or hereinafter may be used for a manufacturing a rotary cutter or any other wear object for example mining drill bits or can punch tooling.

The present invention is further illustrated by the following non-limiting examples.

### Examples

Table 1 outlines the different compositions used for mixing WC-Co cemented carbide. For all of these tests, the mixing was done in two steps using an Eirich Mixer, model RO2VAC. Firstly, the tungsten carbide (WC), cobalt (Co), chromium carbide (Cr₃C₂), carbon (C) powders were mixed together. In tests 3 to 12, the TEA and/or PEI were also added in this step. The constituents were mixed by turning the rotor at 270 rpm whilst the vacuum was applied and then the first step of mixing was done for 20 minutes at 4500 rpm. Distilled water was added at a minimal amount to maintain a temperature of 50°C when the temperature of the powder started to rise.

In the second mixing step, the dry organic constituents (PEG) were added and mixed in at 1500 rpm under vacuum until the temperature reached approximately 70°C and all the PEG had melted, this took approximately 3 minutes. For tests 1 and 2, the TEA was also added at this step. The organic solvents, olaic acid and/or mono propylene glycol (MPG) were then also added and the mixing continued so that a dough was formed. The mixer was turned off when the rotor speed slowed down due to the viscosity of the material.

Samples from tests 1-12 were taken prior to the addition of the organic binders. A small amount of PEG 300 was added and the samples pressed to form 8x7x24mm compacts and then sintered at 1450°C at 50 Bar pressure. The sintered samples were mounted in resin and polished with 180 and then 220 µm grit. The porosity of the samples was examined under an optical microscope and assessed according to ISO standard 4505.

As can be seen in table 1 the A type porosity has significantly reduced in tests 3-12, where the dispersing agent was added in the first mixing step compared to tests 1 and 2, where the dispersing agent was added in the second mixing step.

The samples were then etched using Murikami's reagent for 4 minutes and then examined again under an optical microscope to assess the homogeneity of the microstructure. Tests 1 and 2 yielded cemented carbide bodies with microstructures which contained large clusters of enlarged hard metal grains and large binder lakes. For example figures 1 and 2 show the microstructure of the cemented carbide body produced from test 1. Figure 1 shows a cluster of grains which all have a grain size diameter of >5× the average hard metal grain size. The cluster measures approximately 14 µm across at the widest section. Figure 2 shows binder lakes in the sample, one with a diameter of approximately 3.4 µm and the other with a diameter of approximately 4.1 µm, both greatly exceeding a diameter of 5 x the average hard metal grain size.

Figures 3 and 4 show examples of the microstructure for cemented carbide bodies from tests 3 and 8 respectively. It can be seen that the microstructures have good grain size uniformity, no clusters of enlarged hard metal grains and no binder lakes.

**Table 1**

| **Constituents (wt%)** | **Test 1** | **Test 2** | **Test 3** | **Test 4** | **Test 5** | **Test 6** | **Test 7** | **Test 8** | **Test 9** | **Test 10** | **Test 11** | **Test 12** |
|---|---|---|---|---|---|---|---|---|---|---|---|---|
| WC004 | 82.22 | 0 | 82.47 | 82.12 | 82.48 | 82.15 | 82.39 | 0.00 | 0.00 | 0.00 | 0.00 | 0.00 |
| WC008 | 0 | 82.22 | 0.00 | 0.00 | 0.00 | 0.00 | 0.00 | 82.49 | 82.13 | 82.50 | 82.17 | 82.41 |
| Co | 9.21 | 9.21 | 9.22 | 9.18 | 9.22 | 9.18 | 9.21 | 9.22 | 9.18 | 9.22 | 9.18 | 9.21 |
| Cr₃C₂ | 0.46 | 0.46 | 0.46 | 0.46 | 0.46 | 0.46 | 0.46 | 0.46 | 0.46 | 0.46 | 0.46 | 0.46 |
| C | 0.05 | 0.02 | 0.05 | 0.05 | 0.05 | 0.05 | 0.05 | 0.03 | 0.03 | 0.03 | 0.03 | 0.03 |
| PEG | 5.3 | 5.3 | 5.3 | 5.3 | 5.3 | 5.3 | 5.3 | 5.3 | 5.3 | 5.3 | 5.3 | 5.3 |
| Solvent | 2.67 | 2.67 | 1.92 | 1.92 | 1.92 | 1.92 | 1.92 | 1.92 | 1.92 | 1.92 | 1.92 | 1.92 |
| TEA added in first (dry) mixing step | 0 | 0 | 0.10 | 0.50 | 0.00 | 0.00 | 0.10 | 0.10 | 0.50 | 0.00 | 0.00 | 0.10 |
| TEA added in second mixing step | 0.09 | 0.09 | 0.00 | 0.00 | 0.00 | 0.00 | 0.00 | 0.00 | 0.00 | 0.00 | 0.00 | 0.00 |
| PEI added in first (dry) mixing step | 0 | 0 | 0.00 | 0.00 | 0.09 | 0.46 | 0.09 | 0.00 | 0.00 | 0.09 | 0.46 | 0.09 |
| Porosity | A06B 00C0 0 | A06B 00C0 0 | A02B 02C0 0 | A02B 00C0 0 | A00B 06C0 0 | A00B 04C0 0 | A02B 00C0 0 | A00B 02C0 4 | A00B 02C0 2 | A00B0 2C02 | A00B0 2C02 | A00B02 C02 |

## Claims

1. A method of manufacturing a cemented carbide and/or cermet comprising the steps of:
a) providing a powder comprising metal carbide(s) and binder metal(s) and optionally metal nitride(s);
b) mixing the powder composition provided by step a) under vacuum before
c) adding at least one organic binder to the powder composition;
d) mixing the at least one organic binder with the powder composition under vacuum and raising the temperature to a predetermined temperature and keeping the temperature for a predetermined time until the organic binder has melted;
e) subjecting the obtained mixture of step d) to forming and sintering processes;
wherein one or more dispersing agents is added to the powder composition in step a) and wherein one or more cooling agents is added to the powder composition in step b).

2. The method according to claim 1, wherein cemented carbide comprises more than or equal to 70 wt% tungsten carbide and not more than or equal to 30 wt% of at least one other metal carbide and/or metal nitride selected from titanium carbide, tantalum carbide, tantalum nitride, titanium nitride, niobium carbide, vanadium carbide, molybdenum carbide, chromium carbide and mixtures thereof.

3. The method according to claim 1, wherein cermet comprises titanium carbide, titanium nitride, tungsten carbide, tantalum carbide, tantalum nitride, niobium carbide, vanadium carbide, molybdenum carbide, chromium carbide and a mixture thereof.

4. The method according to any of the previous claims, wherein that binder metal(s) is selected from cobalt, molybdenum, iron, chromium or nickel and a mixture thereof.

5. The method according to any of the previous claims, wherein that the mixing is performed by using a planetary mixer.

6. The method according to any of the previous claims, wherein one or more organic solvents is added in step d).

7. The method according to any of the previous claims, wherein the obtained mixture of step d) is dried after the forming and prior to sintering in step e).

8. The method according to any of the previous claims wherein the one or more dispersing agents is selected from triethanol amine (TEA) or polyethylene imine (PEI) and a mixture thereof.

9. The method according to any of the previous claims, wherein in the forming is performed by using extrusion, pressing operation or injection moulding.

## Patentansprüche

1. Verfahren zum Herstellen eines Hartmetalls und/oder Cermets, das die folgenden Schritte umfasst:
a) Bereitstellen eines Pulvers, das Metallcarbid(e) und Bindemetall(e) und optional Metallnitrid(e) umfasst,
b) Mischen der in Schritt a) bereitgestellten Pulverzusammensetzung unter Vakuum vor
c) Zugabe mindestens eines organischen Bindemittels zu der Pulverzusammensetzung,
d) Mischen des mindestens einen organischen Bindemittels mit der Pulverzusammensetzung unter Vakuum und Erhöhen der Temperatur auf eine vorbestimmte Temperatur und Halten der Temperatur für eine vorbestimmte Zeit, bis das organische Bindemittel geschmolzen ist,
e) Unterziehen der erhaltenen Mischung aus Schritt d) einem Formgebungs- und Sinterungsprozess,
wobei der Pulverzusammensetzung in Schritt a) ein oder mehrere Dispergiermittel zugesetzt werden, und
wobei der Pulverzusammensetzung in Schritt b) ein oder mehrere Kühlmittel zugesetzt werden.

2. Verfahren nach Anspruch 1, wobei das Hartmetall mehr als oder gleich 70 Gew.-% Wolframcarbid und nicht mehr als oder gleich 30 Gew.-% mindestens eines anderen Metallcarbids und/oder Metallnitrids, ausgewählt aus Titancarbid, Tantalcarbid, Tantalnitrid, Titannitrid, Niobcarbid, Vanadiumcarbid, Molybdäncarbid, Chromcarbid und Mischungen davon, umfasst.

3. Verfahren nach Anspruch 1, wobei das Cermet Titancarbid, Titannitrid, Wolframcarbid, Tantalcarbid, Tantalnitrid, Niobcarbid, Vanadiumcarbid, Molybdäncarbid, Chromcarbid und eine Mischung davon umfasst.

4. Verfahren nach einem der vorhergehenden Ansprüche, wobei das/die Bindemittelmetall(e) aus Kobalt, Molybdän, Eisen, Chrom oder Nickel und einer Mischung davon ausgewählt wird/werden.

5. Verfahren nach einem der vorhergehenden Ansprüche, wobei das Mischen unter Verwendung eines Planetenmischers durchgeführt wird.

6. Verfahren nach einem der vorhergehenden Ansprüche, wobei in Schritt d) ein oder mehrere organische Lösungsmittel zugesetzt werden.

7. Verfahren nach einem der vorhergehenden Ansprüche, wobei die in Schritt d) erhaltene Mischung nach dem Formen und vor dem Sintern in Schritt e) getrocknet wird.

8. Verfahren nach einem der vorhergehenden Ansprüche, wobei das eine oder die mehreren Dispergiermittel ausgewählt sind aus Triethanolamin (TEA) oder Polyethylenimin (PEI) und einer Mischung davon.

9. Verfahren nach einem der vorhergehenden Ansprüche, wobei die Formgebung durch Strangpressen, Pressen oder Spritzgießen erfolgt.

## Revendications

1. Procédé de fabrication d'un carbure cémenté et/ou d'un cermet, comprenant les étapes consistant à :
a) fournir une poudre comprenant un ou des carbures métalliques et un ou des métaux liants, et en option un ou des nitrures métalliques ;
b) mélanger la composition de poudre fournie par l'étape a) sous vide avant
c) d'ajouter au moins un liant organique à la composition de poudre ;
d) mélanger le liant organique, au moins au nombre de un, avec la composition de poudre sous vide et élever la température jusqu'à une température prédéterminée et maintenir la température pendant une durée prédéterminée jusqu'à ce que le liant organique ait fondu ;
e) soumettre le mélange obtenu de l'étape d) à des procédés de formage et de frittage ;
dans lequel un ou plusieurs agents de dispersion sont ajoutés à la composition de poudre à l'étape a) et dans lequel un ou plusieurs agents de refroidissement sont ajoutés à la composition de poudre à l'étape b).

2. Procédé selon la revendication 1, dans lequel le carbure cémenté comprend au moins 70 % en poids de carbure de tungstène et au plus 30 % en poids d'au moins un autre carbure métallique et/ou nitrure métallique choisi parmi le carbure de titane, le carbure de tantale, le nitrure de tantale, le nitrure de titane, le carbure de niobium, le carbure de vanadium, le carbure de molybdène, le carbure de chrome et des mélanges de ceux-ci.

3. Procédé selon la revendication 1, dans lequel le cermet comprend du carbure de titane, du nitrure de titane, du carbure de tungstène, du carbure de tantale, du nitrure de tantale, du carbure de niobium, du carbure de vanadium, du carbure de molybdène, du carbure de chrome et un mélange de ceux-ci.

4. Procédé selon l'une quelconque des revendications précédentes, dans lequel ledit ou lesdits métaux liants sont choisis parmi le cobalt, le molybdène, le fer, le chrome et le nickel, ou un mélange de ceux-ci.

5. Procédé selon l'une quelconque des revendications précédentes, dans lequel le mélange est effectué en utilisant un mélangeur planétaire.

6. Procédé selon l'une quelconque des revendications précédentes, dans lequel un ou plusieurs solvants organiques sont ajoutés à l'étape d).

7. Procédé selon l'une quelconque des revendications précédentes, dans lequel le mélange obtenu de l'étape d) est séché après le formage et avant le frittage à l'étape e).

8. Procédé selon l'une quelconque des revendications précédentes, dans lequel le ou les agents dispersants sont choisis parmi la triéthanolamine (TEA), le polyéthylèneimine (PEI) ou un mélange de ceux-ci.

9. Procédé selon l'une quelconque des revendications précédentes, dans lequel le formage est effectué en utilisant une extrusion, une opération de pressage ou un moulage par injection.
